

June 14, 1960

M. SCHOR

2,940,196

STRIPPABLE LABEL

Filed Aug. 15, 1958



INVENTOR  
*Milton Schor*

BY  
*John Jackson, Jr.*  
ATTORNEYS

2,940,196

## STRIPPABLE LABEL

Milton Schor, Havertown, Pa., assignor to A. H. Wirz, Inc., Chester, Pa., a corporation of Pennsylvania

Filed Aug. 15, 1958, Ser. No. 755,259

1 Claim. (Cl. 40—2)

The present invention relates to collapsible tubes provided with strippable labels, to methods of producing strippable labels on collapsible tubes, and to compositions for use in such labels.

A purpose of the invention is to obtain better strippability of strippable labels on collapsible tubes and the like, especially at low plasticizer contents, and under low temperature conditions, and generally to improve strippability.

A further purpose is to produce a strippable label which has better wetting properties for label printing ink, which adheres better to the ink, which permits the ink to dry faster, and which makes the ink more resistant to smudging especially immediately after printing.

A further purpose is to improve the low temperature flexibility of a strippable label, so that it will remain in intimate contact with the metal of the collapsible tube and conform to the collapsible tube when it is squeezed or otherwise pinched in normal collapsible tube use, but will still, at temperatures likely to be encountered in service, readily strip and peel from the collapsible tube.

A further purpose is to produce a strippable label on a collapsible tube or the like which is more resistant to soapy water, more resistant to moisture and more resistant to alkali.

A further purpose is to secure a strippable label which is more resistant to scuffing and abrasion and generally tougher.

Further purposes appear in the specification and claim.

In the drawing I illustrate a collapsible tube provided with a strippable label which has been printed with label information, and embodies the principles of the invention.

The single figure illustrates such a collapsible tube in perspective.

Describing in illustration but not in limitation and referring to the drawing:

In accordance with my United States patent application Serial No. 372,963, filed August 7, 1953, for Strippable Label and Method, now Patent No. 2,855,707, issued October 14, 1958, I illustrate and describe a strippable label which is provided on a collapsible tube and is useful especially in the pharmaceutical trade to permit the retail pharmacist to remove the label where required without the difficulty and annoyance of soaking and removing a paper label, or optionally to sell the produce over the counter and allow the label to remain and identify the product to the consumer.

There may be many reasons for requiring optional removal of a label. It may be desired to sell the product on a prescription and provide information or instructions which are peculiar to the particular patient. It also may be desired to avoid transmitting to the patient information which appears on the original label, as for example, so as not to unduly alarm the patient, or create some misapprehension in the mind of the patient from the initial label information.

Accordingly, strippable labels having information

printed thereon have been supplied on several million collapsible tubes.

The present invention is concerned with the improvement of strippable labelling, overcoming certain deficiencies and difficulties which have existed in the prior art.

By the present invention it is possible to produce plastic labels capable of application to collapsible tubes or the like by spraying, dipping or roller coating, which remain in intimate contact with the surface of the collapsible tube when the collapsible tube is pinched or squeezed, but which have definitely improved properties in several other respects. One important feature of the present invention is that the desired properties can be obtained with smaller plasticizer contents. This aids in getting better ink adherence due to increased wetting of the film to ink, faster drying of the ink, and greater resistance of the ink to smudging, especially immediately after printing by roller printing methods.

It is also possible by the invention to greatly improve the strippability of the label at low temperatures, down to as low as zero degrees F. and even much below this temperature. In the prior art practice the tendency has been for the labels to become less easily strippable at low temperatures, but this is not true of the preferred composition in the present invention.

The invention also makes possible the production of strippable labels which are more resistant to abrasion and scuffing incident to shipment, sale and use.

The invention also assures that the label will tend to remain intimately associated with the collapsible tube when the collapsible tube is pinched, bent or rolled even down to very low temperatures, well below zero degrees F.

Another important aspect of the invention is that the strippable labels have greater resistance to moisture, to soapy water, to alkalies and to chemicals generally. They resist sunlight and weathering, and are resistant to fungi. They resist grease and perspiration.

In accordance with the invention, the collapsible tube, which should be preferably warm and dry, and may be unlabelled or provided with the usual adhering rotary printed label, is coated with a layer of resin in accordance with the invention, using preferably roller coating techniques, but permissibly dipping or spraying.

At the time the label is applied, the end of the collapsible tube which is to be crimped is open and the collapsible tube is truly cylindrical and normally positioned on a cylindrical mandrel. The collapsible tube after coating is normally carried through a dryer at elevated temperature, suitably in the range from 100 to 400 degrees F., although the collapsible tube can dry in air at ambient temperature. The drying time is 255 degrees F. is preferably about 10 minutes.

After drying, the strippable label on the collapsible tube desirably has a thickness from 0.0004 to 0.001 inch.

Once the strippable label has dried, the strippable label is rotary printed, desirably using the usual collapsible tube printing techniques, and applying any suitable label information, such as the name of the product, the instructions for use, the dosage, the maker's name, and the like.

One of the great advantages of the present invention as already mentioned is that the usual label printing inks adhere better, dry faster and are more resistant to smudging when applied on the strippable label of the present invention.

The basis for the strippable label of the present invention is a copolymer of vinyl chloride and vinyl acetate of medium molecular weight. A preferred embodiment contains about 10 percent by weight of vinyl acetate, and has a molecular weight of about 90,000. The range of vinyl acetate is suitably from 7 to 13 percent,

the balance being vinyl chloride, copolymerized. A desirable form of this material is Exxon 450, made by Firestone Tire and Rubber Company, containing about 10 percent vinyl acetate.

In addition to the copolymer resin referred to, I use as a plasticizer a dialkyl sebacate, having a carbon chain length between 6 and 20 carbon atoms, and most desirably dioctyl sebacate. Other examples are dioctadecyl sebacate and didodecyl sebacate.

The quantity of plasticizer used based on the weight 10 of the copolymer resin will vary from 10 to 75 percent and will preferably be in the range from 10 to 24 percent and most desirably from 15 to 24 percent, the optimum being about 20 percent.

In addition I use a solvent which of course evaporates in the process of drying of the strippable label. The preferred solvent is isophorone. I can however use other solvents, including any of the recognized ketone solvents, such as methylethyl ketone, ethyl butyl ketone, and methyl isobutyl ketone. I can also use dimethyl formamide, nitrofuran, and nitroparaffin. Where the odor is not objectionable, I can use cyclohexanone.

As a means of reducing the expense, I can where desired incorporate a solvent diluent, a preferable form being super high flash naptha, which desirably has a kaubutanol factor of 95 and a boiling point for 20 percent of the content at 350 degrees F.

In making up the composition, the copolymer resin and the plasticizer are incorporated with the solvent and the solvent diluent. It is usually necessary to mix under mechanical agitation for a time of the order of one-half hour before the ingredients are thoroughly dissolved. It is not however ordinarily necessary to use heat for solution.

I illustrate in the drawing a completed collapsible tube according to the invention. The tube 20 has a generally cylindrical body 21, a discharge end 22 which receives a cap, a shoulder 23 and an opposite pinched end closure 24. The body is surrounded by a strippable label 25 produced in accordance with the invention and having rotary printed thereon labelling information 26.

The relation of the collapsible tube to the strippable label is unusual. When the solvent evaporates the coating which forms the strippable label shrinks and draws itself smooth into intimate contact with the outer surface of the body of the collapsible tube. An intimate association between the coating and the collapsible tube occurs, since when the user squeezes or presses the collapsible tube and bends it or flattens it down, the label conforms to and remains against the metal surface of the collapsible tube, and does not detach itself from or "bag" away from the collapsible tube. On the other hand, the label does not have appreciable adhesion to the collapsible tube because when the user desires to detach the label he merely needs to rip it with his finger nail or with an instrument as shown at 27, and the label will readily peel away from the collapsible tube and will permit complete removal of the label. Underneath the collapsible tube surface or its label is clean and free from any strippable label material.

As already explained, the capability of the label of remaining with the collapsible tube when the collapsible tube is pinched at low temperature is greatly improved in the present invention, especially when the sebacates are used as plasticizers.

Furthermore, the collapsible tube provided with the label can be washed in soapy water or alkaline detergents without danger of harm to the label or the printing.

In some cases it is desirable to render the strippable label opaque, and this can be done by pigment, which should preferably be inserted to a concentration of about two pounds per gallon of the coating liquid, suitable pigments being paint grades of titanium dioxide, barium sulphate, lithopone, iron oxide, chromic oxide, phthalocyanine green or blue or the like.

The following examples are typical of clear strippable label formulas in accordance with the present invention:

*Example I*

|                                                              | Parts by weight |
|--------------------------------------------------------------|-----------------|
| Copolymer of vinyl chloride and vinyl acetate<br>(Exxon 450) | 20.00           |
| Plasticizer (dioctyl sebacate)                               | 2.00            |
| Super high flash naptha                                      | 39.00           |
| Solvent (isophorone)                                         | 39.00           |

*Example II*

|                                                              |       |
|--------------------------------------------------------------|-------|
| Copolymer of vinyl chloride and vinyl acetate<br>(Exxon 450) | 20.00 |
| Plasticizer (dioctyl sebacate)                               | 9.00  |
| Super high flash naptha                                      | 35.00 |
| Solvent (isophorone)                                         | 36.00 |

*Example III*

|                                                              |       |
|--------------------------------------------------------------|-------|
| Copolymer of vinyl chloride and vinyl acetate<br>(Exxon 450) | 20.00 |
| Plasticizer (dioctyl sebacate)                               | 15.00 |
| Super high flash naptha                                      | 30.00 |
| Solvent (isophorone)                                         | 35.00 |

25 The compositions of these various materials all are useful in accordance with the present invention, but they differ somewhat in the particular properties when used for strippable materials.

Example I with the low content of plasticizer is more 30 difficult to start stripping because of greater resistance to penetration, but once stripping begins it strips very easily and cleanly, and usually in one piece. On the other hand, the formulation of Example II and particularly the formulation of Example III penetrates more easily to start stripping, but once stripping begins the composition has more the consistency of chewing gum, is likely to separate in several pieces and therefore is likely to take longer to strip.

As far as ink adherence (printability) is concerned, this 35 is better with the composition of Example I than it is with the composition of Example III.

The resistance to moisture, soap and alkali are slightly better for Example I than for Example III.

On the other hand, the low temperature flexibility in 40 case the collapsible tube is squeezed at low temperature is somewhat better with Example III.

In some cases it is preferable to print the collapsible tube 45 in the normal manner first with label information, and then to apply the strippable label over the printed collapsible tube and then subsequently print the strippable label with different label information. Then the retailer can select whether he will leave the strippable label in place or remove it prior to sale. In some cases this procedure can be applied over only a portion of the length of the collapsible tube, using the strippable label to mask only a partial printed label.

In view of my invention and disclosure variations and 50 modifications to meet individual whim or particular need will doubtless become evident to others skilled in the art, to obtain all or part of the benefits of my invention 55 without copying the product and method shown, and I, therefore, claim all such insofar as they fall within the reasonable spirit and scope of my claim.

Having thus described my invention, what I claim as 60 new and desire to secure by Letters Patent is:

In combination with a collapsible tubular metal container 65 having a body, an end adapted to be closed by crimping, and an opposite discharge end, a thin coating of a film forming resin composition extending entirely around the body of said tube between the opposite ends of said tube and terminating lengthwise short of at least one of said ends, said coating itself remaining intimately associated with the metal surface of said tube throughout the area of the tube covered by said coating and being capable of remaining intact when the tube and coating are 70 75

deformed at the same point, said coating further having peeling properties when broken, lifted, and pulled, said coating having printed matter on the outside surface thereof and accordingly serving as a label until broken and peelably removed, and said coating consisting of a copolymer of vinyl chloride and vinyl acetate, and from 10 percent to 24 percent on the weight of a long chain dialkyl compound having a carbon chain length between

6 and 20 carbon atoms, combined with the sebacic acid group, as a plasticizer.

References Cited in the file of this patent

UNITED STATES PATENTS

|           |       |       |               |
|-----------|-------|-------|---------------|
| 2,825,159 | Schor | ----- | Mar. 4, 1958  |
| 2,855,707 | Schor | ----- | Oct. 14, 1958 |